

## United States Patent Office

2,769,690

Patented Nov. 6, 1956

1

2,769,690

## INHIBITING CORROSION OF FERROUS METALS

John E. Mahan, Bartlesville, Okla., and Robert A. Stahl, Kansas City, Kans., assignors to Phillips Petroleum Company, a corporation of Delaware

No Drawing. Application June 23, 1952,  
Serial No. 295,118

10 Claims. (Cl. 23—157)

This invention relates to methods of reducing corrosion of ferrous metals by dilute aqueous solution of nitric acid. In one of its aspects the present invention relates to a composition of matter of reduced corrosiveness with respect to ferrous metals.

Dilute aqueous nitric acid solutions are used extensively, in commercial operations such as in pickling baths, bleaching operations, and the purification and preparation of metals and their compounds. It is known that dilute solutions of nitric acid when in contact with apparatus constructed of ferrous metals exert a deleterious corrosive effect thereupon. As a consequence of this corrosive action, recourse had been had to the use of noble metals, highly expensive alloys, or to equally expensive lined equipment that are not appreciably attacked. This corrosion situation has resulted in placing an uneconomical cost disadvantage upon handling of such materials.

It is therefore an object of the present invention to provide a method of reducing the rate of corrosion of ferrous metals by a dilute aqueous solution of nitric acid to an extremely low rate.

It is a further object of this invention to provide dilute aqueous nitric acid solutions of reduced corrosiveness with respect to ferrous metals.

Another object of this invention is to provide a method for rendering dilute aqueous nitric acid solutions which normally corrode ferrous metals rapidly, much less corrosive in their action upon said ferrous metals.

Further and additional objects of this invention will be readily apparent from the disclosure and discussion herein below.

It has been disclosed in the prior art that ammoniacal solutions, such as ammoniacal ammonium nitrate, which are corrosive to ferrous metals with which they may come in contact, may be rendered less corrosive by the addition thereto of small amounts of such materials as thiocyanates and thiourea, sodium arsenite and others. It appears therefore that the materials heretofore employed are effective for inhibiting the corrosiveness of basic solutions toward ferrous metals.

We have now surprisingly found that dilute aqueous solutions of nitric acid which are much more highly corrosive to ferrous metals than the aforementioned basic solutions, can be effectively inhibited in their corrosive action toward ferrous metals by adding selected sulfur-containing compounds to said acid solutions. We have further surprisingly found that alkali metal and ammonium arsenites in combination with the selected sulfur-containing compounds used in the present invention provide dilute aqueous nitric acid solutions of still further reduced corrosiveness. This is especially surprising in view of the fact that we have found, in the case of sodium arsenite, that sodium arsenite alone provides no reduction in the corrosiveness of dilute aqueous nitric acid solution toward ferrous metals.

By the term "ferrous metals," we mean to include within the scope of this invention high carbon and low

2

carbon steels generally, boiler plate, cast iron, malleable cast iron, wrought iron, puddled wrought iron, austenitic steel, and copper-, molybdenum- and nickel-containing steels or combinations thereof. In fact, all ferrous metals which are corrodible by dilute nitric acid solutions are included within the scope of this invention.

In accordance with this invention the corrosion of ferrous metals by a dilute aqueous solution of nitric acid can be substantially reduced by adding to said nitric acid solution a compound or mixture of compounds from the class represented by the general formula



wherein R is a radical selected from the group consisting of hydrogen and alkyl groups containing not to exceed four carbon atoms, and wherein R<sub>1</sub> is a radical selected from the group consisting of hydrogen, alkyl groups containing not to exceed four carbon atoms, and a thioamide radical, and wherein R and R<sub>1</sub> together form heterocyclic ring structures containing up to five members consisting of carbon and nitrogen, said compounds containing not more than seven carbon atoms per molecule. Typical compounds applicable to use in the present invention include: thiourea; 1,3-dimethyl-2-thiourea; 1,3-diethyl-2-thiourea; 1-methyl-3-isopropyl-2-thiourea; 1-methyl-3-tert-butyl-2-thiourea; 1-ethyl-3-tert-butyl-2-thiourea; 1-ethyl-2-thiourea; 1-methyl-2-thiourea; ethylidene thiourea having the following structural formula:



35 ethylene thiourea; N,N-(tetra methyl-ethylene)-thiourea; 2,4-dithiobiuret; 1-methyl-2,4-dithiobiuret; 1-ethyl-2,4-dithiobiuret; 1-propyl-2,4-dithiobiuret; 1-n-butyl-2,4-dithiobiuret; 1-tert-butyl-2,4-dithiobiuret and the like. Thiourea and dithiobiuret are available commercially. The 40 substituted thioureas may be made in any of the following ways: (1) by heating the thiocyanate of primary or secondary amines; (2) by adding hydrogen sulfide to a di-substituted cyanamide; (3) by adding ammonia or primary or secondary amines to mustard oil (isothiocyanates) RNCS; (4) by heating primary amines with carbon disulfide; and (5) by heating thiophosgene with amines.

The arsenite compounds employed in our invention are those selected of the group consisting of sodium arsenite, potassium arsenite, lithium arsenite, ammonium arsenite.

50 The quantity of our inhibitors which can be incorporated to reduce the rate of corrosion may vary from a very small percentage upward, depending upon the degree of corrosiveness of the nitric acid solutions to be inhibited. The degree of corrosiveness of nitric acid solutions is a function of such factors as concentration and temperature. Dilute aqueous acid solutions of up to 50 weight percent nitric acid can be inhibited by the incorporation therein of our inhibitors. However, the preferred range of concentration of our inhibitors is from 0.05 to 2.0 weight percent of the selected sulfur-containing compounds, and from 0 to 1.95 weight percent of the selected arsenite. The total weight percent of inhibitor, whether combined or alone not to exceed 2.0 per cent.

Our invention has specific application to aqueous solutions of nitric acid containing preferably not to exceed 15 weight percent of nitric acid at temperatures below about 150° F., more preferably at temperatures below about 100° F. At these low temperatures very small amounts of our inhibitors effectively inhibit the corrosiveness of the acid to ferrous metals.

The following examples are intended to be illustrative

of underlying principles and should not be construed as unduly limiting our invention.

#### EXAMPLE I

The results of the following tests demonstrate that the compounds disclosed in the present invention substantially reduce the corrosiveness of aqueous solutions of nitric acid on ferrous metals. The test procedure involved following the weight loss of metal strips submerged in inhibited and uninhibited or control test solutions in tightly stoppered, wide mouthed, four-ounce bottles. The test solution was 15 weight percent aqueous nitric acid.

Plates of low carbon steel were used as test specimens. The plates were cut from a sheet of  $\frac{1}{16}$ " steel and were approximately  $\frac{3}{8}$ " wide and 3" long having a total area of 2.67 square inches exposed to the corrosive solution. A coating of mill scale was removed from each specimen by a wire buffering wheel before the test and the plates were clean and shiny.

The bottles were filled with 15 weight per cent aqueous nitric acid, approximately 120 cc. weighed quantities of the inhibitor being tested were added and the bottles thoroughly shaken until the inhibitors were completely dissolved. The test specimens were pickled for five minutes in 36 weight percent hydrochloric acid before the tests were started. The weighed plates were placed in the solutions where they remained for two hours under static conditions at a temperature of 75° F. The plates were then removed, washed with water, dried, and weighed to determine the extent of corrosion as a function of time.

The results expressed in terms of corrosion in inches per day, are tabulated below.

#### Corrosion of low carbon steel at 75° F. caused by 15% nitric acid

(Corrosion rates expressed in inches per day)

| No.    | Inhibitor              | Percent Inhibitor Added | Corrosion, In./Day, 0-2 Hrs. | Percent Reduction in Corrosion Rate |
|--------|------------------------|-------------------------|------------------------------|-------------------------------------|
| 1..... | Control.....           | 0                       | 0.192                        | .....                               |
| 2..... | do.....                | 0                       | 0.198                        | .....                               |
| 3..... | Thiourea.....          | 0.10                    | 0.0025                       | 98.72                               |
| 4..... | do.....                | 0.10                    | 0.0038                       | 98.05                               |
| 5..... | Ethylene Thiourea..... | 0.10                    | 0.0023                       | 98.82                               |

#### EXAMPLE II

The test procedure of Example I was repeated using inhibitors of the present invention at a temperature of 100° F. The results, expressed in terms of corrosion in inches per day, are tabulated below:

#### Corrosion of low carbon steel at 100° F. caused by 15% nitric acid

(Corrosion ratio expressed in inches per day)

| No.    | Inhibitor              | Percent Inhibitor Added | Corrosion, In./Day, 0-2 Hrs. | Percent Reduction in Corrosion Rate |
|--------|------------------------|-------------------------|------------------------------|-------------------------------------|
| 1..... | Control.....           | 0                       | 0.192                        | .....                               |
| 2..... | do.....                | 0                       | 0.198                        | .....                               |
| 3..... | Thiourea.....          | 0.10                    | 0.0089                       | 95.44                               |
| 4..... | do.....                | 0.10                    | 0.0090                       | 95.38                               |
| 5..... | Ethylene Thiourea..... | 0.10                    | 0.0079                       | 95.95                               |

#### EXAMPLE III

In addition to the tests reported in the previous examples a qualitative test was made wherein a 0.10 weight percent solution of dithiobiuret in 15 weight percent nitric acid was employed as test solution. The appearance of the metal strips was observed for evidence of corrosion. At a concentration of 0.10 percent for

dithiobiuret, good protection was provided over a period of two hours.

#### EXAMPLE IV

In addition to the tests described in the previous examples wherein sulfur-containing compounds of the present invention were used alone, tests were also conducted wherein they were used in combination with sodium arsenite. The test procedure of Example I was employed and the tests were conducted at 75° F. The results, expressed in terms of corrosion in inches per day, are recorded in the following table.

TABLE 1

Corrosion of low carbon steel at 75° F. caused by 15% nitric acid

| No.    | Inhibitor              | Percent Inhibitor Added | Corrosion, In./Day, 0-2 Hrs. | Percent Reduction in Corrosion Rate |
|--------|------------------------|-------------------------|------------------------------|-------------------------------------|
| 20     |                        |                         |                              |                                     |
| 1..... | Control.....           | 0                       | 0.192                        | .....                               |
| 2..... | do.....                | 0                       | 0.198                        | .....                               |
| 3..... | Sodium arsenite.....   | 0.10                    | 0.198                        | None                                |
| 4..... | Thiourea.....          | 0.10                    | 0.0025                       | 98.72                               |
| 5..... | do.....                | 0.10                    | 0.0038                       | 98.05                               |
| 25     | Thiourea.....          | 0.10                    | 0.0003                       | 99.85                               |
| 6..... | (Sodium arsenite.....) | 0.10                    | 0.0003                       | 99.85                               |
| 7..... | (Thiourea.....)        | 0.10                    | 0.0016                       | 99.18                               |
|        | (Sodium arsenite.....) | 0.10                    | 0.0016                       | 99.18                               |

The above results show that sodium arsenite alone provides no reduction in corrosion when compared to the control. However, in combination with thiourea the reduction is even more pronounced than that provided by thiourea alone.

While this invention has been described and exemplified in terms of its preferred embodiments those skilled in the art will readily appreciate that modification can be made without departing from the spirit or scope of the invention.

We claim:

1. A process for reducing the corrosion of ferrous metals by a dilute aqueous nitric acid solution, which comprises incorporating in said acid solution both a compound represented by the general formula



wherein R is a radical selected from the group consisting of hydrogen and alkyl groups containing not to exceed four carbon atoms, and wherein R<sub>1</sub> is a radical selected from the group consisting of hydrogen, alkyl groups containing not to exceed four carbon atoms, and a thiocarbonyl radical, and wherein R and R<sub>1</sub> together form heterocyclic ring structures containing up to five members consisting of carbon and nitrogen, said compound containing not more than seven carbon atoms per molecule, and an arsenite selected from the group consisting of sodium arsenite, potassium arsenite, lithium arsenite and ammonium arsenite, in amounts sufficient to decrease the rate of corrosion of a ferrous metal by said acid solution.

2. A process for reducing the corrosion of ferrous metals by an aqueous acid solution containing about 15 weight percent nitric acid, which comprises incorporating into the said acid solution from 0.05 to 2.0 weight percent of a compound represented by the general formula



wherein R is a radical selected from the group consisting of hydrogen and alkyl groups containing not to exceed four carbon atoms, and wherein R<sub>1</sub> is a radical selected

from the group consisting of hydrogen, alkyl groups containing not to exceed four carbon atoms, and a thioamide radical, and wherein R and R<sub>1</sub> together form heterocyclic ring structures containing up to five members consisting of carbon and nitrogen, said compound containing not more than seven carbon atoms per molecule, and from 0 to 1.95 weight percent of an arsenite selected from the group consisting of sodium arsenite, potassium arsenite, lithium arsenite and ammonium arsenite, the total weight percent of inhibitor not exceeding 2.0 percent.

3. A process for reducing the corrosion of ferrous metals by an aqueous acid solution containing about 15 weight percent nitric acid, which comprises incorporating in said acid solution from 0.05 to 2.0 weight percent of a compound selected from the group consisting of thiourea, ethylene thiourea, and dithiobiuret, and from 0 to 1.95 weight per cent of sodium arsenite, the total weight percent of inhibitor not exceeding 2.0 percent.

4. A process according to claim 3 in which 0.05 to 1 percent thiourea and 0.05 to 1 percent sodium arsenite are added to the aqueous acid solution.

5. A process according to claim 3 wherein ethylene thiourea is added to said aqueous acid solution.

6. A process for reducing the corrosion of a low-carbon steel by a dilute aqueous nitric acid solution, which comprises incorporating in such acid solution thiourea and sodium arsenite in amounts sufficient to decrease the rate of corrosion of said low-carbon steel by said acid solution.

7. A process for reducing the corrosion of a low-carbon steel by an aqueous acid solution containing about 15 weight percent nitric acid at temperatures up to 200° F., which comprises incorporating in said acid solution from 0.05 to 2.0 weight percent thiourea and from 0 to 1.95 weight percent sodium arsenite, the total weight percent of inhibitor not exceeding 2.0 percent.

8. As a new composition of matter of reduced corrosiveness with respect to ferrous metals, dilute aqueous

nitric acid solution containing a compound represented by the general formula



wherein R is a radical selected from the group consisting of hydrogen and alkyl groups containing not to exceed four carbon atoms, and wherein R<sub>1</sub> is a radical

10 selected from the group consisting of hydrogen, alkyl groups containing not to exceed four carbon atoms, and a thioamide radical, and wherein R and R<sub>1</sub> together form heterocyclic ring structures containing up to five members consisting of carbon and nitrogen, said compound 15 containing not more than seven carbon atoms per molecule, and an arsenite selected from the group consisting of sodium arsenite, potassium arsenite, lithium arsenite and ammonium arsenite, in amounts sufficient to decrease the rate of corrosion of a ferrous metal by said 20 solution.

9. As a new composition of matter, a dilute aqueous acid solution containing about 15 weight percent nitric acid and thiourea and sodium arsenite in amounts sufficient to decrease the rate of corrosion of a ferrous metal 25 by said solution.

10. As a new composition of matter, a dilute aqueous nitric acid solution containing ethylene thiourea and sodium arsenite in amounts sufficient to decrease the rate of corrosion of a ferrous metal by said solution.

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

3480

3485

3490

3495

3500

3505

3510

3515

3520

3525

3530

3535

3540

3545

3550

3555

3560

3565

3570

3575

3580

3585

3590

3595

3600

3605

3610

3615

3620

3625

3630

3635

3640

3645

3650

3655

3660

3665

3670

3675

3680

3685

3690

3695

3700

3705

3710

3715

3720

3725

3730

3735

3740

3745

3750

3755

3760

3765

3770

3775

3780

3785

3790

3795

3800

3805

3810

3815

3820

3825

3830

3835

3840

3845

3850

3855

3860

3865

3870

3875

3880

3885

3890

3895

3900

3905

3910

3915

3920

3925

3930

3935

3940

3945

3950

3955

3960

3965

3970

3975

3980

3985

3990

3995

4000

4005

4010

4015

4020

4025

4030

4035

4040

4045

4050

4055

4060

4065

4070

4075

4080

4085

4090

4095

4100

4105

4110

4115

4120

4125

4130

4135

4140

4145

4150

4155

4160

4165

4170

4175

4180

4185

4190

4195

4200

4205

4210

4215

4220

4225

4230

4235

4240

4245

4250

4255

4260

4265

4270

4275

4280

4285

4290

4295

4300

4305

4310

4315

4320

4325

4330

4335

4340

4345

4350

4355

4360

4365

4370

4375

4380

4385

4390

4395

4400

4405

4410

4415

4420

4425

4430

4435

4440

4445

4450

4455

4460

4465

4470

4475

4480

4485

4490

4495

4500

4505

4510

4515

4520

4525

4530

4535

4540

4545

4550

4555

4560

4565

4570

4575

4580

4585

4590

4595

4600

4605

4610

4615

4620

4625

4630

4635

4640

4645

4650

4655

4660

4665

4670

4675

4680

4685

4690

4695

4700

4705

4710

4715

4720

4725

4730

4735

4740

4745

4750

4755

4760

4765

4770

4775

4780

4785

4790

4795

4800

4805

4810

4815

4820

4825

4830

4835

4840

4845

4850

4855

4860

4865

4870

4875

4880

4885

4890

4895

4900

4905

4910

4915

4920

4925

4930

4935

4940

4945

4950

4955

4960

4965

4970

4975

4980

4985

4990

4995

5000

5005

5010

5015

5020

5025

5030

5035

5040

5045

5050

5055

5060

5065

5070

5075

5080

5085

5090

5095

5100

5105

5110

5115

5120

5125

5130

5135

5140

5145

5150

5155

5160

5165

5170

5175

5180

5185

5190

5195

5200

5205

5210

5215

5220

5225

5230

5235

5240

5245

5250

5255

5260

5265

5270

5275

5280

5285

5290

5295

5300

5305

5310

5315

5320

5325

5330

5335

5340

5345

5350

5355

5360

5365

5370

5375

5380

5385

5390

5395

5400

5405

5410

5415

5420

5425

5430

5435

5440

5445

5450

5455

5460

5465

5470

5475

5480

5485

5490

5495

5500

5505

5510

5515

5520

5525

5530

5535

5540

5545

5550

5555

5560

5565

5570

5575

5580

5585

5590

5595

5600

5605

5610

5615

5620

5625

5630

5635

5640

5645

5650

5655

5660

5665

5670

5675

5680

5685</